

Patented Apr. 25, 1950

2,505,180

# UNITED STATES PATENT OFFICE

2,505,180

## ELECTROLYTE

Alexander M. Georgiev and James J. Campbell,  
Dayton, Ohio, assignors to General Motors Corporation,  
Detroit, Mich., a corporation of Delaware

No Drawing. Application April 2, 1947,  
Serial No. 738,930

2 Claims. (Cl. 175—315)

1

This invention relates to electrolytic condensers and more particularly to improvements in the electrolyte.

The objects of the invention include the provisions of an electrolyte which can be economically produced from relatively inexpensive ingredients and by a relatively simple method not requiring expensive equipment and to provide an electrolyte having relatively low viscosity, having greater penetrating properties thereby facilitating the impregnation of prewound condenser sections, either before or after insertion in unsealed cans, and permitting the use of thin dense paper in the condenser windings and also to provide an electrolyte having physical and chemical stability, thereby permitting the reuse of the same batch of electrolyte until it is entirely consumed.

The objects of the invention include improvements in electrolytic condensers by reason of the use of the improved electrolyte.

Further objects of the present invention will be apparent from the following description of methods of manufacture thereof.

The new electrolyte is the resultant of the combination ethylene glycol, boric acid and ammonium borate, the quantity of ethylene glycol being very large in proportion to the quantities of the other two ingredients.

Satisfactory results can be obtained by using commercial ammonium borate which contains water of crystallization, and hydrous (ortho) boric acid  $H_3BO_3$  or anhydrous boric acid  $B_2O_3$ . The proportions can be:

|                 | Percent      |
|-----------------|--------------|
| Ammonium borate | about 2 to 5 |
| $H_3BO_3$       | 3 to 18      |
| Ethylene glycol | 95 to 80     |

$H_3BO_3$  at 10% and ethylene glycol at 85% is preferred. The mixture is preferably agitated and heated in an open vessel, preferably between 230° and 300° F. until the solids are dissolved and the resistivity at 85° F. is above 1000 ohms per cubic centimeter and preferably not greater than 4000 ohms per cubic centimeter. The specific viscosity of the electrolyte so prepared is at 20° F. in the range of 1.0 to 1.5, for example, as compared with the viscosity of water at 60° F. The electrolyte is very fluid at 200° F. Its pH is in the range of 4 to 5.

Another method consists of mixing boric acid, either  $H_3BO_3$  or  $B_2O_3$  (anhydrous), with ethylene glycol in about the proportions of 5 to 20% boric acid and 95 to 80% ethylene glycol. This mixture is agitated and heated, preferably between 230° and 300° F., for a time sufficient to dissolve the solids and, eventually, expel excess water and to obtain a certain resistance, for example, about 200,000 ohms per cubic centimeter at 85° F. It is desirable to obtain a cer-

tain high resistance as a starting point for the step which follows. Then enough ammonia gas (usually about .2% to .6% of the total weight of the electrolyte) is caused to bubble through the cooled composition of boric acid and ethylene glycol to reduce the resistivity to the desired value. The resistivity at 85° F. is in the range of 1000 to 4000 ohms per cubic centimeter. The exact value depends on the particular voltage rating and application of the condenser, 1500 to 3000 ohms per cubic centimeter being typical. Its pH is of the order of 4 to 5.

In either case an electrolyte is obtained comprising ethylene glycol and the reaction products of ethylene glycol with boric acid and ammonium borate. While the electrolyte has a rather milk acid reaction, it does not attack the aluminum electrodes of the electrolytic condenser and has excellent film-forming and film-sustaining properties. The ammonia in combination reduces the resistivity and, as a glycol compound of ammonium borate, provides a film-maintaining substance.

The second method has the advantages of greater economy in materials used, saving in time and a more convenient and precise control of the composition as to proportions of ingredients, presence of water and electrochemical characteristics: pH, resistivity, film-forming and film-sustaining properties. The resistivity of the electrolyte is primarily a function of water content and of ammonia content. For the best results from the film-forming point of view, the desired resistivity should be obtained by separately controlling these factors. This separate control is obtained by following the second method which requires evaporation of water from the mixture of ethylene glycol and boric acid before ammonia gas is added in order to obtain a predetermined resistance of high value; and then the addition of ammonia gas to reduce the high resistance to a predetermined moderate resistance. This is preferred to the evaporation which concurrently expels water and ammonia. By using the second method very small portions of the ingredients are lost in the course of evaporation. Since evaporation takes place prior to the bubbling of ammonia, none of the ammonia will be lost.

*Résumé of important novel features of the electrolyte*

The electrolyte is easily and quickly prepared, because a comparatively small amount of solids is readily dissolved in a great proportion of solvent. Since little water is present in the composition to begin with, only moderate evaporation is required to reduce the water content to the small, desirable quantity. In some cases no evaporation at all will be required.

Due to the great percentage of solvent in this electrolyte and its extreme fluidity (it is about as fluid as the pure ethylene glycol alone) it provides a uniform and continuous wetting and coverage of the aluminum electrodes. The resulting advantages are: rapid and thorough impregnation of prewound sections, either before or after placing in unsealed cans, possibility of using thin, dense paper in winding the sections, which contributes to the compactness of the condensers, uniformity and efficiency in the operation of the total electrode area, since a homogeneous electrolyte is distributed all over the aluminum surfaces. Easy diffusion of the electrolyte throughout the section, which tends to equalize the temperature, averts the formation of hot spots in the winding and thus helps it to withstand electrical overloading. The high percentage of ethylene glycol, which is a plasticizer, prevents the drying out of the condenser in case of overheating and exposure to the air. Drying out is the common weakness of condensers made with the conventional viscous or semi-solid glycol electrolytes. The formation of lumps of salt, as ordinarily found in other electrolytes made of the same ingredients, is minimized or avoided.

The elimination of waste is even more pronounced in the course of impregnation of condenser sections, because the electrolyte does not cake, i. e. does not form insoluble precipitates, and can be reused indefinitely, until completely consumed. Any precipitate which may eventually be formed on cooling is redissolved on reheating. Other electrolytes made of the same ingredients and heretofore used have a strong tendency to cake and become unsuited for reuse. Large proportions of the electrolyte are therefore discarded from time to time, resulting in appreciable material losses. It has been experienced heretofore that, after repeated heating of the electrolyte, cakes or substantially solid lumps would be formed. Such caking would take place when several batches of condenser sections are impregnated in succession in the same bath. Such caking rendered the electrolyte unsuitable because it interfered with the proper impregnation of the condenser sections. It necessitated the discarding of the electrolyte batch thus causing waste of material and increasing the cost of production. The present electrolyte possesses physical and chemical stability thereby enabling the same batch to be reused until entirely consumed. Waste of materials is avoided with the result that the cost of production is reduced.

The outstanding penetrating properties of the present electrolyte permit the impregnation of prewound sections without resorting to the use of complicated, costly equipment. They also markedly shorten the time required for impregnation. Due to these penetrating properties it is also practicable to impregnate the condenser sections after they have been inserted but not sealed in their containers. This procedure results in an appreciable saving in labor, in the uniform absorption of electrolyte and expansion (swelling) of the sections in the course of impregnation and in the elimination of the handling of impregnated sections, which may entail their contamination. This method of impregnation in containers also provides an automatic, firm and lasting positioning of the section in the can, thus making wedging (a slow and costly operation) unnecessary.

*Characteristics of the condensers impregnated with the new electrolyte*

1. Low leakage current, low power factor, high capacity per unit area of foil.
- 5 2. Good breakdown characteristics across the line.
3. Effective and uniform cooling while in operation, due to the diffusion of the fluid electrolyte. Avoidance of hot spots.
- 10 4. Resistance to drying out when subjected to prolonged heating (when current allowed to flow in condenser for a long time), and or exposed to the air. This is due to the great proportion of ethylene glycol versus solid constituents (boric acid, ammonium borate) used in the preparation of the electrolyte.
5. Compactness, because thin, dense paper spacers can be used in winding of condenser section.
- 20 6. Easier and better assembling of condensers due to practicability of impregnating sections after their insertion in cans when this fluid electrolyte is used.

While the form of embodiment of the present invention as herein disclosed, constitutes a preferred form, it is to be understood that other forms might be adopted, all coming within the scope of the claims which follow.

What is claimed is as follows:

1. The method of making a low viscosity, substantially anhydrous electrolyte for electrolytic condensers, which comprises; mixing 5% to 20% boric acid with 95 to 80% ethylene glycol, by weight, heating the mixture at a temperature between 230° F. to 300° F. for a time sufficient to completely dissolve the solids and to substantially eliminate water, cooling the reaction mixture, and then passing ammonia gas therethrough in quantities sufficient to bring the resistivity of the solution at 85° F. to within the range of 1000 to 4000 ohms per cubic centimeter and for controlling the pH value of the solution to a figure of between 4 and 5, whereby a stable, fluid electrolyte is formed.

2. A low viscosity, substantially anhydrous and stable electrolyte for use in electrolytic condensers, consisting of an anhydrous, unsaturated solution of the reaction mixture of boric acid and ethylene glycol wherein the boric acid varies between 5% and 20%, which solution has been ammoniated by passing ammonia gas therethrough in quantities sufficient to produce a resistivity within the electrolyte of from 1000 to 4000 ohms at 85° F. a viscosity at 200° F. of from 1 to 1 1/2 as compared to the viscosity of water at 60° F. and an acidity having a pH of from 4 to 5.

ALEXANDER M. GEORGIEV.  
JAMES J. CAMPBELL.

**REFERENCES CITED**

The following references are of record in the file of this patent:

**UNITED STATES PATENTS**

| Number    | Name           | Date          |
|-----------|----------------|---------------|
| 1,815,768 | Georgiev ----- | July 21, 1931 |
| 1,891,207 | Ruben -----    | Dec. 13, 1932 |
| 1,909,506 | Ruben -----    | May 16, 1933  |
| 1,924,711 | Edenburg ----- | Aug. 29, 1933 |
| 2,031,128 | Raines -----   | Feb. 18, 1936 |
| 2,062,543 | Waterman ----- | Dec. 1, 1936  |
| 2,196,057 | Clark -----    | Apr. 2, 1940  |